

## UNITED STATES PATENT OFFICE

2,516,737

## HOT-ROLLED BINARY ZINC-TITANIUM ALLOY

Thomas C. Wilson, Washington, D. C., assignor to The New Jersey Zinc Company, New York, N. Y., a corporation of New Jersey

No Drawing. Application January 15, 1944,  
Serial No. 518,418

2 Claims. (Cl. 148—32)

1

This invention relates to binary zinc-titanium alloys, and particularly to the alloys disclosed in my copending United States patent application Ser. No. 460,933, filed October 6, 1942, now abandoned. The present invention is concerned with the working of such alloys and contemplates certain improvements in the mechanical working and especially the rolling of such alloys.

The binary zinc-titanium alloys disclosed in my aforementioned patent application contain from 0.01% to 1.6%, and preferably from 0.05% to 0.3%, titanium, with the balance zinc, preferably high-grade zinc, although zinc of the grade commonly used in commercial rolled zinc may be used. These alloys are conveniently manufactured by first preparing a zinc-titanium hardener by adding about 4% of titanium metal to molten zinc and holding under a boric acid cover, with frequent stirring, at 750° C. until the titanium is dissolved. The desired titanium content in the binary zinc-titanium alloy is then readily obtained by adding the calculated amount of this hardener to a predetermined weight of molten zinc.

The binary zinc-titanium alloys of my aforementioned patent application, when transformed to sheet or strip by suitable rolling procedure, possess high creep resistance (resistance to cold flow), namely, resistance to prolonged static loads well below the ultimate limit. Cold working or rolling tends to decrease the creep resistance of these alloys, but their normal high creep resistance can be substantially restored by subse-

5 loys at temperatures of from 190 to 300° C., temperatures of from 200 to 235° C. giving very satisfactory results. The hot rolling or mechanical working of the invention may be a finishing operation consisting of say three or more passes through the rolls, and may be preceded by either cold or hot rough rolling.

10 Creep resistance or creep rate may be measured and directly expressed as the percent elongation or creep of a standard test piece during a unit of time, say one day, when subjected to a dead load of, say, 8000 pounds per square inch (p. s. i.) at constant room temperature (25° C.). When the creep rate is so expressed, the lower values (percent/days) represent the higher creep resistance. I prefer to express the creep resistance as the inverse creep rate which is the number of units of time, say days, required to produce an elongation or creep of one percent (days/percent), whereby the more creep resistant alloy (or material) has the higher inverse creep rate.

15 The following Table I shows the mechanical properties and superior inverse creep rates of three (Nos. 1, 2 and 3) hot-rolled zinc-titanium alloys of the invention, contrasted with a zinc-copper alloy containing 1% copper. The zinc-titanium alloys were hot rolled to 0.02" in a 12" diameter mill with a final coil temperature of about 200° C. The bars rolled quite easily and 20 produced strip of good surface quality. The rolled strips were subjected to the normal routine 25 mechanical property tests including determinations of creep rate.

Table I

| No.    | Analyzed<br>Per Cent<br>Ti Balance<br>Zn <sup>1</sup> | Test<br>Gauge,<br>In. | Sclero-<br>scope<br>Hard-<br>ness | Dy-<br>namic<br>Ductil-<br>ity, In. | Tem-<br>per-<br>Per<br>Cent | 180° Bends <sup>2</sup> |                 | Tensile Strength,<br>Lb./Sq. In. |                 | Tensile Elon-<br>gation, Per<br>Cent in 2" |                 | Inverse Creep Rates, Days<br>Per Cent<br>Elongation,<br>With Grain Stress |                    |                    |
|--------|-------------------------------------------------------|-----------------------|-----------------------------------|-------------------------------------|-----------------------------|-------------------------|-----------------|----------------------------------|-----------------|--------------------------------------------|-----------------|---------------------------------------------------------------------------|--------------------|--------------------|
|        |                                                       |                       |                                   |                                     |                             | With<br>Grain           | Across<br>Grain | With<br>Grain                    | Across<br>Grain | With<br>Grain                              | Across<br>Grain | 8,000<br>p. s. i.                                                         | 12,000<br>p. s. i. | 15,000<br>p. s. i. |
| 1----- | 0.05                                                  | 0.023                 | 19                                | 0.320                               | 36                          | 2½                      | 2               | 19,500                           | 27,600          | 33.2                                       | 13.3            | 24.8                                                                      | 0.055              | 0.0039             |
| 2----- | 0.12                                                  | 0.021                 | 20                                | 0.300                               | 37                          | 3                       | 2               | 20,100                           | 29,900          | 29.5                                       | 12.0            | 190.0                                                                     | 1.05               | 0.023              |
| 3----- | 0.23                                                  | 0.022                 | 22                                | 0.295                               | 40                          | 4                       | 2               | 21,300                           | 30,000          | 28.3                                       | 11.3            | 1,120.0                                                                   | 4.66               | 0.077              |
| 4----- | 1% <sup>3</sup> Cu                                    | 0.018                 | 17                                | 0.280                               | 40                          | 3½                      | 2               | 23,700                           | 30,000          | 35.0                                       | 8.7             | 1.95                                                                      | 0.16               | No Test            |

<sup>1</sup> Alloys prepared with 99.99% pure zinc.<sup>2</sup> Values represent the diameter of the bend in multiples of sheet thickness. Small values indicate better bending properties.<sup>3</sup> Hot rolled, analogous to Zn-Ti treatment.<sup>4</sup> Tests not run to the usual 6-per cent total elongation. Values recorded represent the slope of the line joining the origin of the curve of time vs. elongation with the final recorded point-values probably lower than true values.

quent heat treatment such, for example, as by annealing for five minutes at a temperature of about 275° C. Cold working, at least during the last stages of the rolling, imparts to the metal certain advantages, especially with respect to the drawing properties.

In the course of my investigations, I have found that the aforementioned binary zinc-titanium alloys when hot rolled into sheet or strip form can be readily fabricated. Based on that discovery, the present invention involves mechanically working or rolling these zinc-titanium al-

55 loys at temperatures of from 190 to 300° C., temperatures of from 200 to 235° C. giving very satisfactory results. The hot rolling or mechanical working of the invention may be a finishing operation consisting of say three or more passes through the rolls, and may be preceded by either cold or hot rough rolling.

The data in Table I shows the remarkable creep resistance of the hot-rolled alloys of the invention. At moderate loads (e. g. 8000 p. s. i.), the creep resistance of these alloys is astonishingly high, particularly in the case of the alloy containing 0.23% titanium (No. 3).

As hereinbefore stated, I have found that the temperature of rolling exercises a very great effect upon the creep resistance of the rolled strip. 60 With a rolling temperature around 160° C., the inverse creep rate of a zinc-titanium alloy containing 0.12% titanium was 0.033 (days/percent)

under a load of 12,000 p. s. i. With a rolling temperature around 190° C. the inverse creep rate of the same alloy was 0.72, and with a rolling temperature of around 210° C. the inverse creep rate was 1.76. The effect of rolling temperature upon the creep resistance of the rolled alloy is shown in the following tables in which Table II gives the schedule of the rolling operations of 5 specimens of a zinc-titanium alloy containing 0.12% titanium, and Table III gives the inverse creep resistance rate of the resulting rolled strips. The preliminary or rough rolling schedule was the same for each specimen (A to E) and reduced the specimens from slabs 7" x 14" x 1 1/4" to a gauge of approximately 0.09" in ten passes through the rolls. The first horizontal line of Table II is the temperature of the rolls, the second horizontal line is the starting temperature of the alloy specimens, D and E being preheated in order to attain the higher final coil temperatures. The specimens were given three passes (four for A) through the rolls to effect a reduction in gauge from about 0.09" to about 0.02" (0.015" for C). The last horizontal line of the table is the final coil temperature of the rolled strip after the final rolling pass.

Table II

| A<br>140-160° C.<br>Room | B<br>170-190° C.<br>Room | C<br>170-190° C.<br>Room | D<br>170-190° C.<br>140° C. | E<br>170-190° C.<br>140° C. |
|--------------------------|--------------------------|--------------------------|-----------------------------|-----------------------------|
| 0.090                    | 0.091                    | 0.089                    | 0.093                       | 0.090                       |
| 0.073                    | 0.064                    | 0.070                    | 0.065                       | 0.065                       |
| 0.044                    | 0.036                    | 0.042                    | 0.035                       | 0.037                       |
| 0.028                    | 0.018                    | 0.015                    | 0.018                       | 0.019                       |
| 0.018                    |                          |                          |                             |                             |
| 161° C.                  | 188° C.                  | 211° C.                  | 230° C.                     | 234° C.                     |

Table III

| Specimen | Final coil<br>Temper-<br>ature | Inverse<br>Creep Rate,<br>days/percent<br>12,000 p. s. i. |
|----------|--------------------------------|-----------------------------------------------------------|
| A        | 161                            | 0.033                                                     |
| B        | 188                            | 0.72                                                      |
| C        | 211                            | 1.76                                                      |
| D        | 230                            | 5.45                                                      |
| E        | 234                            | 6.71                                                      |

The influence of hot rolling upon the creep resistance of the zinc-titanium alloys is further illustrated by Table IV, in which the hot rolled alloy (0.12 titanium) is contrasted with the cold rolled alloy, and with hot and cold rolled zinc-copper alloy (1% copper).

Table IV

| Alloy         | Rolled    | Sclero-<br>scope<br>Hard-<br>ness | Tensile<br>Strength,<br>p. s. i. | Elonga-<br>tion,<br>Per<br>Cent | Inverse<br>Creep<br>Rate,<br>8,000 p. s. i.<br>Days/Per<br>Cent |
|---------------|-----------|-----------------------------------|----------------------------------|---------------------------------|-----------------------------------------------------------------|
| Zn-Ti.....    | Hot.....  | 21                                | 19,700                           | 34                              | 100                                                             |
| Zn-Ti.....    | Cold..... | 15                                | 17,900                           | 39                              | 1.2                                                             |
| Zn-1% Cu..... | Hot.....  | 17                                | 23,700                           | 35                              | 1.9                                                             |
| Zn-1% Cu..... | Cold..... | 25                                | 28,000                           | 54                              | 2.3                                                             |

From the foregoing examples, it will be seen that the hot rolled or worked alloys of the invention possess remarkably high creep resistance. The line of demarcation between cold and hot rolling, so far as the effect upon creep resistance is concerned, seems to be in the neighborhood of 160-180° C. With rolling temperatures below that temperature range, the creep resistance is not un-

usual. With rolling temperatures above that temperature range, a significant and sharp increase in creep resistance is attained. The contemplated conditions of hot rolling can be established by preheating the alloy or by heating the rolls so that the thermal conditions during rolling impart a final temperature of 190 to 300° C. to the alloy passing from the final roll (final coil temperature). It is not necessary, and in practice not likely, that the contemplated hot rolling temperature be maintained during each pass of the complete rolling schedule. The advantages of the invention are satisfactorily attained where the final coil temperature is within the contemplated hot rolling temperature range.

The data in Table IX reveal the unusual effect in the zinc-titanium alloy of cold rolling effecting a softening and weakening as compared with hot rolled material. The work hardening revealed in the 1% copper alloy is, of course, the normal result.

Photomicrographs of the hot and cold rolled zinc-titanium alloy of the invention show the metal to be apparently free of cold working in the cold rolled state, an observation that is consistent with the physical properties of the metal.

Redraw tests showed that as many as four redraws could be made without intermediate anneals, and with at least 95% recovery of unfractured material. Thus, it is evident that the alloy does not work harden. Another interesting property of the alloy is the appearance of a high population of basal planes normal to the rolling plane and lying in the rolling direction.

Contrary to experience with zinc, the zinc-titanium alloy has been found not to grow excessively large grains when annealed. Anneals up to 24 hours' duration at temperatures up to 400° C. failed to produce relatively coarse grain structures. Moreover, it has been found that ductility and other properties are not harmed by annealing and, significantly, the high creep resistance noted in the hot rolled alloy which was sharply reduced by cold working was found to be largely restored by suitable heat treatment.

I claim:

1. A binary zinc-titanium alloy product containing from 0.01% to 1.6% titanium and having been subjected to a finishing treatment consisting of hot rolling at a temperature within the range of 190° C. to 300° C.

2. A binary zinc-titanium alloy product containing from 0.05% to 0.30% titanium and having been subjected to a finishing treatment consisting of hot rolling at a temperature within the range of from 200° C. to 235° C.

THOMAS C. WILSON.

#### REFERENCES CITED

The following references are of record in the file of this patent:

#### UNITED STATES PATENTS

| Number    | Name           | Date          |
|-----------|----------------|---------------|
| 979,393   | Rossi .....    | Dec. 20, 1910 |
| 1,020,512 | Rossi .....    | Mar. 19, 1912 |
| 1,835,450 | Anderson ..... | Dec. 8, 1931  |
| 1,888,567 | Pierce .....   | Nov. 22, 1932 |
| 2,048,288 | Pierce .....   | July 21, 1936 |
| 2,169,441 | Winter .....   | Aug. 15, 1939 |
| 2,317,179 | Daesen .....   | Apr. 20, 1943 |

#### OTHER REFERENCES

Metals Handbook, 1939 edition, pages 1737, 1765; pub. by American Society for Metals, Cleveland, Ohio.

**Certificate of Correction**

July 25, 1950

Patent No. 2,516,737

THOMAS C. WILSON

It is hereby certified that error appears in the printed specification of the above numbered patent requiring correction as follows:

Column 2, line 9, for "precent" read *percent*; line 51, for "shows" read *show*; column 4, line 16, for "Table IX" read *Table IV*; and that the said Letters Patent should be read as corrected above, so that the same may conform to the record of the case in the Patent Office.

Signed and sealed this 17th day of October, A. D. 1950.

[SEAL]

THOMAS F. MURPHY,  
*Assistant Commissioner of Patents.*